

## UNITED STATES PATENT OFFICE

ALBERT CHARLES BARTLETT AND JOHN WALTER RYDE, OF WEMBLEY, ENGLAND

## ELECTRIC DISCHARGE TUBE

No Drawing. Application filed November 17, 1927, Serial No. 234,030, and in Great Britain November 25, 1926.

This invention relates to electric gas discharge tubes and more particularly to cathodes for such tubes.

For many purposes it is important that the potential required to start a discharge through the tube and the potential required to maintain through it a discharge once started should both be as low as possible. A low starting potential is desirable in order that the discharge may start on the usual supply circuits; a low running potential is desirable in order that the energy dissipated in the tube when a given current passes through it shall be as small as possible. It is known that both these potentials can be reduced concurrently by substituting highly electropositive substances for ordinary metals as cathodes; accordingly it has been proposed to coat a cathode composed of ordinary metals with a layer of electropositive substances, such as the alkali or alkaline earth metals, or the alkaline earth oxides such as are used for thermionic emission. All such substances when exposed to the atmosphere react with it to form less electropositive substances which have little or no effect in reducing the discharge potential. Accordingly in the manufacture of discharge tubes with such "sensitive" cathodes, it is necessary to prevent the access of air to the vessel between the formation of the sensitive surface and the final sealing off.

We have found that cathodes characterized by low running potentials can be prepared which will retain their properties, even after exposure to the atmosphere. Such cathodes can be made by causing suitable compounds of the alkaline earth metals to react with nickel, iron or certain of their alloys in virtue of a suitable heat treatment. But cathodes of this type are not "sensitive" in quite the same sense as those coated with the alkaline metals, because the starting potential is not appreciably lower than that obtained with ordinary cathodes; only the running potential is lower. However, for some purposes the starting potential is unimportant and only the running potential important. Thus in biphasic rectifiers of the known type in which two anodes are closely associated with the

same cathode enclosed in a single vessel, the potential available to start the discharge is double the peak potential of the rectified supply, and is often sufficient even when unsensitized cathodes are used. On the other hand a low running potential is important, because it implies a low energy loss in rectification.

According to the invention cathodes characterized by running potentials appreciably lower than those of the ordinary metals and not appreciably higher than those of the alkali metals and also stable when exposed to the atmosphere are obtained by coating metallic cathodes of nickel, iron or their alloys by suitable compounds of the alkaline earth metals and subjecting them to a controlled heat treatment, whereby the compound reacts with the metallic cathodes forming a new compound which contains both the alkaline earth metal and the nickel or iron.

It must be understood that the process is entirely different from that by which cathodes of the alkaline earth oxides are prepared, as in the original Wehnelt process, by heating an alkaline earth compound on a metallic support. In the Wehnelt process the layer remaining on the metallic support was substantially pure alkaline earth oxide and did not consist of a compound containing both the alkaline earth metal and that of the support. The formation of such complex compounds is essential to our invention.

Again it has been suggested several times that the success of various methods of preparing oxide cathodes for thermionic discharge vessels depends on a reaction between the oxide coating and the underlying metal. But it does not appear to have been suggested that cathodes prepared in this manner would be valuable in gas discharge vessels, nor would many of these methods be applicable to bodies of the shape required.

A preferred method of preparing cathodes according to this invention is as follows. The electrodes which may be made of nickel, are coated with a layer of moistened barium nitrate and carefully dried by warming them. The electrodes so coated are then placed in a

vacuum furnace of any suitable form and heated carefully up to about 750° C. for about half an hour and then cooled. During the heating process the barium nitrate coating reacts with the nickel and changes its colour. The heating is so controlled that the coating produced is of a reddish brown colour. If the temperature to which the electrodes are heated is too low the colour of the coating is usually black and crystalline, whilst if the temperature is raised too high the colour is either lead grey or white and the coatings so produced are not satisfactory. The exact composition of the reddish brown barium compound has not been ascertained. Electrodes which have been produced by the controlled heat treatment described above may be exposed to air during their assembly in electric discharge tubes without any adverse effect on their subsequent behaviour. To complete the manufacture of a discharge tube, the tube after assembly of the electrodes is evacuated and baked in a known manner, a charge of rare gas admitted and an electric discharge passed to heat the electrodes to a dull red heat until no further evolution of gas occurs. The charge of gas is then pumped out, the tube filled with a suitable gas and sealed off in the usual known manner.

30 Although it is preferable to carry out the controlled heat treatment of the coated electrodes in a vacuum furnace, this is not essential, as it has been found that it is possible to obtain satisfactory results by heating the 35 coated electrodes in air. Further, although nickel electrodes are preferred electrodes of nickel alloys, iron, or iron alloys may also be used.

We claim:—

- 40 1. A process for the manufacture of cathodes for electric gas discharge tubes which comprises coating an electrode containing nickel with barium nitrate, subjecting the coated electrode to a controlled heat treatment to partially decompose the said barium nitrate and to produce a compound which is neither gray nor black but reddish brown.
- 45 2. The manufacture of cathodes according to claim 1, in which the heat treatment consists of heating for half an hour to a temperature of 750° C. in a vacuum furnace.
- 50 3. Cathodes for electric gas discharge tubes comprising a nickel cathode member coated with a reddish brown compound of barium, nickel and oxygen.

ALBERT CHARLES BARTLETT.  
JOHN WALTER RYDE.